

C. Peters,

Mold for Uniting Cast Iron and Steel.

№ 9,578.

Patented Feb. 8, 1853.



Witnesses:

J. M. C. and  
A. B. Beasley

Inventor:

C. Peters

# UNITED STATES PATENT OFFICE.

CHARLES PETERS, OF TRENTON, NEW JERSEY.

## IMPROVEMENT IN MOLDS FOR UNITING STEEL TO CAST-IRON.

Specification forming part of Letters Patent No. 9,578, dated February 8, 1853.

*To all whom it may concern:*

Be it known that I, CHARLES PETERS, of the city of Trenton, in the county of Mercer and State of New Jersey, have invented a new and Improved Case to Molds in which Steel or Wrought-Iron is to be Welded to Cast-Iron; and I hereby declare that the following is a full and exact description thereof.

The nature of my invention consists in forming a solid basis of iron, brick, or other hard material to the mold, with an aperture therein of the shape of the steel or wrought-iron sought to be welded, and thus by means of the said aperture subjecting the steel or wrought-iron while in the mold to the fire until the same is heated to a welding-heat.

To enable others skilled in the art to make use of my invention, I will proceed to describe its construction and operation, reference being had to the accompanying drawing.

My description and drawing relate to the casting of anvils with steel or wrought-iron faces, from which the application of my invention to other articles will be readily understood.

I form a base for my mold of iron, fire-brick, or other solid material the shape of the flask required to mold the anvil. I then form an aperture in the said base the shape of the steel or wrought-iron face of the anvil, but somewhat smaller, so that the steel or wrought-iron will cover the aperture and be exposed on the under side of the case. I also have a rib surrounding the case of the thickness of the steel or wrought-iron face, so as to form a

recess around said steel or wrought-iron. I have also set-screws and loops to retain the steel or wrought-iron in its place. I then daub the recess with molding-sand, so as to prevent the molten iron from passing around the edges of the steel or wrought-iron face and the screws and recess from getting heated. Upon this base thus formed I then build my mold, precisely as molders are accustomed to do, upon the ground. I then place the mold over a furnace level with the ground, so that the solid part of the base shall be on the ground and nothing but the steel or wrought-iron face shall be exposed through the said aperture to the fire. Having obtained a welding-heat I slide the mold off the fire onto a bed of sand, to prevent the steel or wrought-iron from burning. The molten iron is then poured into the mold in any of the modes practiced by founders. I thus dispense with the heating of the steel or wrought-iron face while out of the mold, and also with the formation of a new base for each casting.

What I claim as my invention, and desire to secure by Letters Patent, is—

The use of a solid base to molds in which steel or wrought-iron is to be welded to cast-iron, with an aperture in the same, so that by means thereof the said steel or wrought-iron can be subjected to the heat of the furnace while in the mold.

CHAS. PETERS.

Witnesses:

SAMIL. EVANS,  
A. W. BEASLEY.